

Dec. 22, 1936.

C. OTTO

2,065,288

PROCESS OF COKING COAL

Filed July 1, 1931

3 Sheets-Sheet 1

Fig. 1



INVENTOR  
*Carl Otto*  
BY  
*W. T. Bissell*  
ATTORNEY

Dec. 22, 1936.

C. OTTO

2,065,288

PROCESS OF COKING COAL

Filed July 1, 1931

3 Sheets-Sheet 2

Fig. 2



INVENTOR  
*Carl Otto*  
BY  
*W. F. Busang*  
ATTORNEY

Dec. 22, 1936.

C. OTTO

2,065,288

PROCESS OF COKING COAL

Filed July 1, 1931

3 Sheets-Sheet 3

Fig. 4



Fig. 3



INVENTOR  
*Carl Otto*  
BY  
*M. F. Bissell*  
ATTORNEY

## UNITED STATES PATENT OFFICE

2,065,288

## PROCESS OF COKING COAL

Carl Otto, Essen-Ruhr, Germany

Application July 1, 1931, Serial No. 548,201  
In Germany July 1, 1930

7 Claims. (Cl. 202—23)

The invention has for its object a coking process to be carried into effect in intermittently operating coking chambers in which process at the beginning of the coking period the gases produced are sucked out of the interior of the charge in such a manner that, in addition to a considerably increased yield of light oil and primary tar an improvement of the quality of the coke is attained, more particularly 5 with coal sorts which have only little tendency to baking. With these ends in view, the suction of the gases of distillation produced at the beginning of the coking period from the interior of the charge is carried through in such a manner that formation of a coking seam is avoided or that such formation at least occurs to a very 10 smaller extent than hitherto. The measures taken for this purpose and described herein-after are based on the hypothesis that the coking seam is due to deposition of vaporous products of distillation on coal particles which are 15 cooler than the products.

According to the invention this condensation and deposition of products of distillation is avoided by either notably increasing the velocity 20 of the escaping products of distillation or increasing their temperature beyond their point of condensation, by admixture of hot gases.

Tests have proved that in order to overcome 25 the resistance offered by a coking seam normally formed in a charge a gas pressure is required which may amount to a substantial part of an atmosphere. Hence, in order to prevent formation of the coking seam or to substantially eliminate the noxious effect of a coking 30 seam already formed upon the escapement of the distillation gases, according to the invention the distillation gases are drawn off from the coking chambers, the charge of which is still 35 in the first stage of the coking period, by means of pipes projecting into the charge and under so high a pressure above atmospheric that no higher pressures prevail in the upper gas collecting spaces of the chambers than in the 40 adjacent heating walls. The pressures required for this purpose in accordance with the results of the tests mentioned amount to at least 200 mm. water, but are frequently much higher. Furthermore, as with pressures of this height 45 the walls existing between the heating flues and the coking chambers which are normally made of silica brickwork are no longer gas-tight, and care has to be taken that no substantially lower pressure prevails in the chambers in the 50 vicinity of these walls than in the adjacent heat-

ing flues. Hence, in practice it is necessary to provide a regulating device by which the power of the gas suction is regulated in such a manner, for instance by means of a valve inserted in the suction conduit, that in the vicinity of 5 the chamber side of the walls that separate the coking chambers from the heating flues neither a notably higher nor a notably lower pressure will prevail than on the side of the heating flues. This regulating device is actuated 10 suitably in a manner as to respond to the difference of pressure existing between the upper gas collecting spaces of the coking chambers and the neighboring heating flues. Such a regulating device is required particularly because the resistance the cake offers to the gases 15 passing therethrough considerably varies during the coking period.

A further possibility of avoiding formation of 20 a coking seam or to notably reduce its disadvantageous effect may consist in introducing into the chambers a hot gas which together with the products of distillation generated is sucked off through the above pipes which project into the charge, this mixture of introduced and distillation gas then having such temperature that it has no tendency to condense even when passing through cooler coal masses of the charge.

Furthermore, instead of introducing superheated steam, hot water gas is also well adapted 30 to realize this portion of the invention, and more particularly even water gas the carbon of which has not yet been largely reduced. The water gas may be supplied either by a special producer or better from coking chambers of the 35 same battery in which the charge has already completely burned off and wherein the water gas is produced by blowing in steam. In this way also the hot distillation gases produced in these coking chambers are supplied together with 40 the water gas thus produced therein to the chambers of the same battery in which the charge is still in the first stage of the coking period.

The hot gases or vapors are supplied either 45 through the upper gas collecting spaces of the chamber or better through pipes which likewise project into the charge and have openings which pipes may be designed like those serving to draw off the distillation gases from the chamber. In 50 this manner of operation two seals may be made use of, the one of which through pipes projecting into the charge draws off the distillation gases from the chambers the charge of which is in the first stage of the coking period, while the other 55

or auxiliary seal merely serves to establish a communication between the upper gas collecting spaces of the chambers the charge of which is in the last coking stage and the members that feed these hot gases to the chambers the charge of which is still in the first coking stage.

The suction of the distillation gases as well as the supply of the hot scavenging gases may be effected by known horizontal or vertical pipes. 10 During the last stage of the coking period the suction pipes may also serve for the introduction of steam into the chambers for the generation of the water gas. If vertical suction pipes are to be provided for, these pipes may be introduced into the chamber through apertures that can be completely gas-tightly shut off. These apertures are provided in series in the oven cover in the central plane of the chamber between the charging holes. After the chamber has been 20 filled suitable rods are pushed down into the fresh charge by which rods passages are prepared for the pipes and which preferably are mounted on the larry car of the battery and manipulated from the latter, the whole system of pushing rods 25 and their actuating mechanism advantageously being designed so as to be rocked or lifted into an inoperative position in order to permit easy travel of the larry car. As a matter of course, however, the pushing rods together with an actuating mechanism hereinafter described may be mounted on a special car travelling on the track 30 of the larry car.

After vertical passages have been formed in the charge by the aid of the above pushing rods, 35 the suction pipes are lowered into these passages so as to project partly thereinto. In order to attain the most uniform possible suction in the vertical direction, the vertical suction pipes may have different lengths so as to project into the 40 charge to different depths.

Furthermore, in order to attain a close contact of the coal with the suction pipes, the latter may be introduced into the charge together with the pushing rods. After this introduction the 45 rods are removed while the suction pipes remain in the charge.

The connection of the suction pipes of each chamber with the common high quality gas seal is advantageously established by providing fixed 50 conduits on the apertures of the oven cover which conduits lead to a main above each chamber serving to draw off the whole distillation gases of a chamber and are connected to the primary tar seal, a valve being provided in each 55 of these conduits. These mains may also be connected to the conduit that feeds superheated steam, so that when going over from the suction of primary tar to introduction of steam, only reversal of the valve is required, whilst the apertures in the oven cover can remain closed and gas tight.

In order that the heavy hydrocarbons drawn off during the first stage of the coking period are not exposed to cracking, the temperature in 65 all the conduits must not exceed a determined degree, and the suction means are therefore cooled.

In order to cool the suction device cooling 70 members may be provided in the suction pipes. These cooling members preferably consist in porous cylinders of ordinary or fire clay to which water is fed dropwise in regulatable quantities. The water then evaporates on the large surface 75 of the cylinders to which thus can be given an exactly determined temperature so that the suc-

tion pipes can be kept cool in any desired degree. The pipes must of course not become too cold as otherwise the high boiling hydrocarbons would condense and return to the coking chamber.

5 In order that the invention may be clearly understood and readily carried into effect, an embodiment of the same is illustrated by way of example in the accompanying drawings in connection with a chamber oven adapted for the 10 realization of the process according to the invention.

Figure 1 is a vertical sectional view thru the top of a coking chamber.

Figure 2 is a vertical section thru the top of a 15 chamber showing a form of carrying car for the pusher rods.

Figure 3 is a sectional view through a coking chamber, showing another form of means for carrying out the invention.

20 Figure 4 is a front view of the chamber shown in Figure 3.

Referring first to Figure 1 which is a view of the top portion of a coking chamber, 1 denotes a coking chamber and 1a the coal charge to be 25 coked in the chamber. The chamber is closed by the usual doors 2. Vertical passages 3 in the charge thru which the distillation gases are drawn off during the first stage of the coking period and thru which steam may be later introduced. The larry car 5 travels on the track 4 and through the hoppers 6 of the car coal is supplied to the chamber through the charging holes 7. After opening the closures 8, the pushing rods 23 (shown in Figure 2), are introduced 30 through the apertures 11 provided in the top of the oven. The pushing rods prepare the above passages 3 in the coal charge. After removal of the rods or also directly with their introduction the pipes 9 are suspended from the apertures 40 11 which pipes are arranged in a row in the longitudinal direction of the chamber and serve first to draw off the distillation gases and later on to supply steam. Within the pipes 9 are mounted the above-described cooling members 10. The apertures 11 which enlarge in upward direction, are connected by pipes 12 to a collecting main 13 which according to the position of the valves 14 and 15 is in communication either with the seal 19 or with the steam 45 collecting conduit 17. The valve 14 is automatically controlled in a manner not shown by a controlling mechanism operating in response to the difference of pressure and communicating both with the gas collecting space 18 of a chamber and one of the adjacent heating walls of the 50 said coking chamber.

The gas collecting spaces 18 of all the chambers of a battery are interconnected by a conduit 16 running within the oven cover in the longitudinal direction of the battery which conduit normally is closed by plugs 16'. By means of valves (not shown) the conduit 16 can be shut off from all but one of the gas collecting 55 spaces 18. These other spaces 18 have to be shut off especially when their doors 2 are to be removed in order to push the respective charge. The conduit 16 serves to supply steam after it has been introduced according to the 60 invention thru the pipes 9 during the last stage of the coking period, or a mixture of steam, water gas and distillation gas, to the chambers in which the charge is still in the first coking stage, whereby an accelerated ex- 70 75 80 85 90 95

pulsion of the heavy hydrocarbons is attained. The distillation gases developed during the last coking stage are thus drawn off immediately from every chamber into main 16 and arrive 5 in the seal 19 only by passing through the collecting main 16 and through those chambers the charge of which is still in the first coking stage. By suitably governing the coking process and the provision of a powerful suction in 10 the individual chambers no formation of any coking seam at all occurs, as hitherto, that is the coking seam hitherto formed in the vertical central plane of the charge does not appear. On the contrary, solid coke blocks extending from 15 the one chamber wall to the other are formed. In this way the possibility is given of production of large coke also in very narrow coking chambers, and of a considerable reduction of the duration of the coking period. Furthermore, 20 because of the fact that by the introduction of steam partial cooling of the charge is attained within the chamber, a smaller quantity of heat is lost by the coke later on being quenched; the heat economy of an oven plant 25 designed according to the invention thus being better than hitherto. Finally, this cooling of the coke within the chamber further favors the formation of large coke blocks, as it has been observed that a coke that already has been 30 cooled partly within the chamber forms larger pieces than a coke which is pushed when still in a very hot state.

In Figure 2 is illustrated by a view of a suitable embodiment of a car carrying the system 35 of pushing rods and appurtenant actuating mechanisms.

The illustrated car 20 travels on the track 4 of the larry car of the battery. 23 denotes the pushing rods which are vertically movably arranged in guide tubes 23'. These tubes have 40 longitudinal slots through which project lugs 21 fixed on the respective pushing rods 23 and serving for the attachment of an endless actuating cable or chain 21' which runs on suitable 45 pulleys or sprocket wheels 22, 22'. The pulleys are driven by a motor (not shown) mounted on the car 20. In this way the rods 23 are pushed into the charge or lifted therefrom.

The improvement of the quality of the tar as 50 aimed at by the invention as well as the increased yield of tar and light oil is warranted only if the weakening of the coal is not accompanied by a quick increase of temperature so that the heavy hydrocarbons generated are not 55 exposed to high temperatures. In connection with a slow increase of temperature the invention further provides that the resistance offered to the distillation gases by a coking seam which maybe is formed remains small. To this end 60 according to the invention the heating of the coking chambers is regulated in such a manner that during the distillation when gases are sucked off from the midst of the coke cake, all portions of the charge, including those situated 65 in close vicinity of the heating walls, have a temperature which does not exceed 700° C. While in the manner of operation hitherto employed the coal particles in the vicinity of the heating walls possessed the temperature of 1000° 70 C. usual in the high temperature coking process, whilst much lower temperatures prevailed in the midst of the cake. According to the invention the temperature of the portions of the charge in the vicinity of the heating walls is maintained 75 below 700° C. until the coal has gone over

throughout to plastic state and as long as the distillation gas is still being sucked off from the midst of the coal cake.

The means to be provided for maintaining the temperature of all portions of the charge below 5 700° C. may be of various nature. It is obvious so to heat the heating walls that only little gas is fed during the first hours of the coking period. For this manner of operation, however, it is necessary that the two coking chambers 10 beside a heating wall are emptied and re-filled only in short intervals or that each heating wall is subdivided into two parallel rows of heating flues. It is possible, however, to maintain a uniform heating and to attain nevertheless 15 the desired low temperature of the coal portions situated near the heating wall by providing special cooling channels in these coal portions. Finally, steam may be blown in from the chamber walls into the chamber which steam 20 causes a cooling of the charge both by taking up sensible heat and by its decomposition by the carbon of the charge.

As already explained above, the introduction of hot gases during the first stage of the coking 25 period may take place through horizontal or vertical pipes in lieu of through the upper gas collecting space, which pipes project into the charge.

The Figures 3 and 4 show embodiments of this 30 type; Figure 3 being a fragmentary view through a coking chamber, while in Figure 4 is the corresponding front view. The upper gas collecting spaces of the chambers which are in the last coking stage can be connected with an auxiliary 35 seal from which the hot distillation gases or a mixture of distillation gas, steam and water gas can be supplied to the chambers which are in the first coking stage by special pipes projecting into the charge.

In addition to the seal 24 which by a vertical pipe 25 and a bent pipe 26 is connected to the upper gas collecting spaces of the chambers of a battery and can be shut off therefrom, and to the collecting pipes 27 which likewise can 45 be shut off by valves 28, an auxiliary seal 29 is provided as collecting space for the distillation gases escaping from the gas collecting space during the first stage of the coking period. This auxiliary seal can be shut off from the individual 50 chambers by valves 30 and is likewise connected to vertical pipes 31 extending between the chamber doors which pipes can be shut off by valves 32. Horizontal pipes provided with perforations 55 may be introduced through the chamber doors 33 which pipes, according to whether they are to serve for sucking off the distillation gases or for supplying the hot steam-water gas mixture, are connected with either the ascension pipes 27 or 31, by means of the bent pipes 34.

All or part of the horizontal pipes may be connected to steam collecting conduits (not shown) after the coking process has already made progress, while the ascension pipes 25 remain shut off during the entire coking period. In this case 65 the distillation gases are drawn off from the battery merely through those of the horizontal pipes which through the ascension pipes 27 are in connection with the hydraulic main 24, while from those chambers to which steam is fed 70 through the horizontal pipes the mixture of distillation gas, steam and water gas arrives through the upper gas-collecting space in the auxiliary main 29 from where it is fed through the ascension pipes 31 and the horizontal pipes attached 75

thereto to the coking chambers the charge of which is in the first stage of the coking period, where it acts as scavenging gas and prevents condensation of constituents of the distillation gas and their deposition onto the coal particles and thus formation of a coking seam.

In Figure 3 only three horizontal pipes one above the other are shown, it will, however, be of advantage to provide a greater number of such 10 pipes in order to attain a more uniform penetration of the charge of the hot scavenging gases and a more effective suction of the distillation gases, the mutual distance of the pipes in a vertical direction then being not greater than 15 about half of or the whole width of the chamber.

Should horizontal pipes be used, it is advantageous to alternately dispose between two 20 neighboring chamber doors the ascension pipes serving to draw off the distillation gases and those serving for the supply of the scavenging 25 gases, as illustrated in Figures 3 and 4.

What is claimed is:

1. The batch process of coking coal in a 25 coking chamber provided with heating walls which comprises charging the chamber with coal, providing passages in said charge leading to the interior thereof, externally heating the charge thereby carbonizing the coal, drawing 30 off distillation gases by suction from the interior of the charge thru said passages during the first coking period, and introducing scavenging gas into said chamber during the first coking period, the temperature of said gases being more than 35 500° centigrade.

2. The batch process of coking coal in coking chambers provided with heating walls, which comprises charging the chambers with coal, providing passages in each charge leading to the interior thereof, externally heating the charge thereby carbonizing the coal, drawing off the distillation gases by suction from the interior of each charge thru said passages during the first coking period, and drawing off the gases from 45 chambers during the last coking period and supplying said gases to other chambers in which the charge is in the first coking period.

3. The batch process of coking coal in a coking chamber provided with heating walls, which 50 comprises charging the chamber with coal, providing passages in said charge leading to the interior thereof, externally heating the charge thereby carbonizing the coal, supplying gas to the chamber during the first stage of the coking 55 period therein at a temperature in excess of 500° C., drawing off distillation and supplied gases during the first stage of the coking period from the interior of the charge by suction, and admitting steam to said charge during a later 60 stage of the coking.

4. The batch process of coking coal in coking chambers provided with heating walls which comprises, charging the chambers with coal, providing passages in each charge leading to the interior thereof, externally heating the charge thereby carbonizing the coal, drawing off distillation gases from the interior of the charge of at least one chamber by suction during the first stage of the coking period, admitting steam 65 to said chamber during a later stage of the coking period thereof, drawing off the distillation gases and water gas generated in the chamber in said later stage, and supplying the gases so generated to another chamber in which the 70 charge is in the first stage of the coking period.

5. The batch process of coking coal in coking chambers provided with heating walls, which comprises charging the chambers with coal successively, providing passages in the charge in each chamber leading to the interior thereof, externally heating each charge thereby carbonizing the coal, supplying gas to each chamber during the first coking period of the charge therein, drawing off the distillation and supplied 10 gas from each chamber by suction during the first coking period of the charge therein, introducing steam into the said passages of the charge in each chamber during a later coking period of the charge therein, and withdrawing the gas formed in each chamber during said later coking period, and utilizing the gas withdrawn from chambers during the later coking periods therein as the gas supplied to chambers in which the first charge coking periods are then occurring.

6. A batch process of coking coal in a horizontal coking retort oven structure comprising a plurality of coking chambers and heating walls alternating therewith and formed with openings in the top wall of each chamber distributed 25 along the length of the latter, and with horizontal channels in the upper portion of said structure extending longitudinally of the chambers and individually adjacent to and communicating with the top wall openings of one 30 of said chambers, and formed with a horizontal passage in the upper portion of the structure extending transversely of said chambers and communicating with each chamber at its top, which process comprises successively charging 35 the different chambers with coal so that the coking operations in the different chambers may begin and end at different times, and so as to leave a gas space at the top of each chamber above the charge therein, providing vertical 40 passages in the charge in each oven, one beneath each of the openings in the top wall thereof, connecting each of the top wall openings of each chamber with the subjacent passage by a conduit traversing the said gas space in the 45 chamber, externally heating the charge in each chamber thereby carbonizing the coal therein, drawing off distillation gases by suction from the interior of the charge in each chamber during the first coking period therein, through the 50 passages in the last mentioned charge and the communicating conduits, openings, and channel, and during the final coking period, in each chamber, supplying superheated steam to the charge therein through the said passages in the 55 charge and the communicating conduits, openings, and channel, and regulating the pressures in the gas spaces in the different chambers so as to create a gas flow between the latter through said horizontal passage into and out of each chamber during the first and final coking 60 periods therein, respectively.

7. A process of coking coal in a horizontal coking retort oven structure comprising a plurality of coking chambers and heating walls alternating therewith, which consists in charging the different chambers at different intervals and so as to leave a gas space above the charge and coking the charges therein in approximately the same coking time so that at any one time the coking operations in different chambers are 65 in different stages, withdrawing the distillation gases from each retort during an early stage of the coking operation therein by applying suction to the interior of the charge therein and thereby creating a gas flow to the interior of 70 75

the charge from said space in said retort and the surface of said charge, and passing gases from the said spaces in retorts in which the coking operations are in later stages without significant change in gas pressure into the said spaces of the retorts in which distillation gases are being withdrawn from the interiors of the charges as aforesaid, whereby the gas pressures

at the surfaces of the charges in the different retorts are equalized and the gases passed into retorts in which the coking operations are in their early stage, serve in the last mentioned retorts as scavenging gases drawn into the 5 charges from the surfaces of the latter.

CARL OTTO.